

March 7, 1972

W. M. TUCKER ET AL

3,647,646

METHOD AND APPARATUS FOR ELECTROPLATING CYLINDRICAL OBJECTS

Filed March 4, 1968

2 Sheets-Sheet 1



FIG. 1



FIG. 2

WILLIAM M. TUCKER  
BARRIE M. GARDNER  
JOHN W. HAYFORD  
INVENTORS

BY *Alfred P. Lorenzo*  
*Paul R. Holmes*  
*Walter O. T. Johnson*  
ATTORNEYS

March 7, 1972

W. M. TUCKER ET AL

3,647,646

METHOD AND APPARATUS FOR ELECTROPLATING CYLINDRICAL OBJECTS

Filed March 4, 1968

2 Sheets-Sheet 2



FIG. 3



FIG. 4

WILLIAM M. TUCKER  
BARRIE M. GARDNER  
JOHN W. HAYFORD  
INVENTORS

BY *Alfred P. Lorenzo*  
*Paul P. Holmes*  
*Walter O'F. Hodson*  
ATTORNEYS

3,647,646

**METHOD AND APPARATUS FOR ELECTRO-PLATING CYLINDRICAL OBJECTS**

William M. Tucker, Barrie M. Gardner, and John W. Hayford, Rochester, N.Y., assignors to Eastman Kodak Company, Rochester, N.Y.

Filed Mar. 4, 1968, Ser. No. 710,035

Int. Cl. C23b 5/56, 5/68; B01k 3/00

U.S. CL. 204—25

26 Claims

**ABSTRACT OF THE DISCLOSURE**

In electroplating a cylindrical object which serves as cathode in the plating process and is positioned adjacent to an anode immersed in the plating bath, the object is mounted in such manner that it is only partially submerged and the bath is agitated with sufficient force that the exposed surface of the object is maintained completely awash with the electrolyte solution. Defects in the plating resulting from occlusion of air bubbles or solid particles are thereby minimized and a high plating rate is attained.

**BACKGROUND OF THE INVENTION****(1) Field of the invention**

The invention relates in general to the art of electroplating and in particular to a novel method and apparatus for plating a cylindrical object with a metal coating.

**(2) Description of the prior art**

A variety of methods of effecting the electroplating of cylindrical objects have been proposed heretofore. In certain of these methods, the cylindrical object, which serves as the cathode in the plating process, has been totally immersed within the electrolyte solution and positioned in proximity to a soluble anode, composed of the metal to be used to form the plate, which is also totally immersed within the electrolyte solution. Other plating processes have utilized a similar arrangement but employ an insoluble anode, in which case the plating metal is supplied by the electrolyte solution. In some instances, the cylindrical object has been mounted in a fixed position within the bath, while in other instances it has been subjected to rotary and/or oscillatory movement to effect agitation of the electrolyte solution in the region immediately adjacent the cathode surface. For the production of metal coatings meeting ordinary quality requirements such techniques are generally quite satisfactory. However, where it is necessary to produce a coating which meets very stringent quality standards, such as is the case in nickel plating of steel rolls used as film transport rolls in the manufacture of photographic film, serious difficulties are encountered. In particular, it is found that numerous small pit-like defects are formed in the nickel plating, either as a result of gas bubbles which are trapped on the surface of the roll while plating and subsequently "plated in," i.e. occluded in the plating structure, or as a result of fracture holes which result from the breaking away during subsequent surface grinding operations of tiny protrusions or nodules on the surface of the plating formed when conductive particles such as carbon, nickel sulfide, iron, iron oxide, and the like, fall on the roll surface during plating and become attached. These defects, even though they are very small in size, can cause scratches or gouges in the moving web of film as it passes over the roll and to avoid this problem an effort is usually made to fill in the defects in the plating with plugs of soft nickel, but, as would be apparent, this is a tedious, time-consuming and expensive procedure.

It is also known to the art to electroplate a cylinder

by positioning the cylinder so that it is less than half immersed in the electrolyte solution and providing an anode of arcuate shape mounted within the electrolyte solution directly beneath the cylinder so that it is substantially equidistant from the face of the cylinder at all points. Such processes, exemplified by U.S. Pat. 1,918,627, accomplish plating only within the zone where the cylinder is immersed but utilize relatively high speed rotation of the cylinder about its axis to secure a uniform deposit over the entire face of the cylinder. They are employed where it is not necessary to plate shaft sections at the ends of the cylinder nor to plate the entire end surfaces of the cylinder and find particular utility in production of printing forms utilized in the rotary photogravure process.

It is toward the objective of providing a novel electroplating method and apparatus, capable of plating cylindrical objects at a high rate with metal coatings in which "in plate" defects are substantially eliminated, or at least greatly reduced in number, and adapted to permit plating of shaft sections and end surfaces as well as the face of the cylindrical object, that the present invention is directed.

**SUMMARY OF THE INVENTION**

The present invention comprises a novel method and apparatus for electroplating a cylindrical object with a metal coating which is adapted to use in diverse applications in the electroplating arts where a high quality plating is required. While the invention is specifically described herein with reference to nickel plating of rolls used as film transport rolls in the manufacture of photographic film, it may be utilized in many other electroplating applications, as long as the workpiece is either a cylinder or of a generally cylindrical shape and the plating system is one in which a high degree of agitation of the bath is not detrimental.

In the method of this invention, the cylindrical object which is to be plated is mounted in the electroplating bath in such manner that it is only partially submerged in the electrolyte solution, i.e., so that part of it is below the level of electrolyte solution and the remaining part is exposed. More specifically, the cylinder is mounted in a generally horizontal position so that its longitudinal axis is substantially parallel to the free surface of the electrolyte solution, i.e., the surface of the electrolyte solution when the bath is in a quiescent state, and at such a level that the uppermost point on the cylindrical surface is above the free surface of the electrolyte solution. Depending on the particular requirements of the specific situation involved, the cylinder may be positioned so that its longitudinal axis is coincident with the surface of the electrolyte solution or so that it is above or below such surface, so long as a substantial portion of the cylindrical surface is immersed within the solution. The cylindrical object serves as the cathode in the plating process and an anode, which may be an insoluble anode or a soluble anode composed of the plating metal, is mounted within the bath in close proximity thereto. As the electric potential is impressed across anode and cathode to effect plating, the electrolyte solution is agitated and preferably, the cylindrical object is rotated about its longitudinal axis. The method of effecting agitation is not critical but the solution must be agitated with sufficient force that the portion of the cylindrical object which is exposed, i.e., above the free surface of the solution, is at all times maintained completely awash with the solution, i.e. continuously and completely covered with a layer of the solution. By this means, the cylindrical object is at all times completely surrounded with electrolyte solution which acts to convey the electric current to its surface so as to effect plating at an effective rate over the entire area and yet the

static head of liquid above any point on the upward-facing surface is very low. Rotation of the cylindrical object which is being plated may be effected in a continuous or intermittent manner, as desired, and agitation of the electrolyte solution may be accomplished by any suitable means known to the art such as gas sparging, solution sparging, or the use of mechanical stirring apparatus.

The method of this invention provides a high plating rate and, at the same time, facilitates formation of a high quality plate which is substantially free of defects. The high plating rate achieved is primarily attributable to the fact that the high degree of agitation of the electrolyte solution effectively replenishes metal ions as they are depleted from immediately adjacent the plating surface. Improvement in the quality of the deposit, i.e., freedom from "in plate" defects, is believed to be a result of the fact that rising bubbles in the solution attributable to the sparging, or other agitation, break as they come in contact with the surface of the cylindrical object and release the gas in such manner that it is not entrapped within the plate, as well as the fact that there is little or no opportunity for particles in the plating bath to settle out onto the rotating cylinder since above any point on the upward-facing cylindrical surface there is only a relatively small depth of solution. Moreover, as the rising bubbles reach the surface of the solution and break they violently scrub the face of the cylinder and wash away any solid particles or minute gas bubbles which have temporarily attached themselves to the cylinder and this action also contributes greatly to the elimination of "in plate" defects.

#### BRIEF DESCRIPTION OF THE DRAWINGS

In the drawings:

FIG. 1 is a partial top plan view of electroplating apparatus in accordance with this invention, illustrating particularly the relative positions of the anode and cathode within the plating tank.

FIG. 2 is an end view of the apparatus taken along line 2-2 of FIG. 1, illustrating particularly the position of the cathode relative to the surface of the electrolyte solution.

FIG. 3 is a longitudinal elevation view of the apparatus taken along the line 3-3 of FIG. 1, illustrating particularly the construction of the anode and showing means provided for recirculation, heating, and filtering of the electrolyte solution.

FIG. 4 is a longitudinal elevation view of the apparatus taken along line 4-4 of FIG. 1, illustrating particularly the relative positions within the plating tank of the cathode and the means provided for agitating the electrolyte solution.

#### DESCRIPTION OF THE PREFERRED EMBODIMENT

As shown in the drawings, plating tank 10, which is rectangular in shape and made of steel plate coated on the interior side with an electrically non-conductive, chemically-resistant coating, such as rubber or polyvinyl chloride, is partially filled with electrolyte solution 12. Arranged within tank 10 in two longitudinally extending rows are a series of identical vertically disposed anodes 14, each of which is in the form of a hollow cylinder filled with chunks of electrolytic nickel and is completely immersed within electrolyte solution 12. A total of ten anodes 14 are shown and these are arranged so that there are five in each row positioned so they are equally spaced from one another. Anodes 14 are made of titanium and have perforated walls adapted to retain the nickel chunks while admitting electrolyte solution 12 into the interior of the cylinder and thereby into contact with the nickel. Positioned between the rows of anodes 14 is a longitudinally extending, horizontally disposed, cylindrical roll 16 which serves as the cathode in the electroplating process. Roll 16 is made of steel and, after being plated with

nickel, is to be used as a film transport roll in the manufacture of photographic film. At each end of roll 16, shaft sections 18 extend a short distance beyond the end of the roll.

The dimensions of anodes 14 and roll 16 can be of any reasonable magnitude, for example, anodes 14 can be two feet high and a few inches in diameter and roll 16 can be five feet in length and a few inches in diameter. In the drawings there are five anodes 14 in each row positioned at substantially equal increments along the length of roll 16 but a lesser or greater number of anodes may be used depending on the relative sizes of the anodes and the roll being plated. Moreover, in practice at the same time a number of rolls arranged within the tank in several parallel rows, with each row being made up of two or more rolls linked together.

As illustrated in FIGS. 2, 3, and 4, anodes 14 are suspended in electrolyte solution 12 by means of anode hangers 20 carried by anode support rods 22 and roll 16 is supported in position adjacent anodes 14 by cathode hangers 24 which engage shaft sections 18 at each end of roll 16 and are carried by cathode support rod 26. Anode support rods 22 are fixedly secured to the end walls of plating tank 10 by braces 28 and cathode support rod 26 is similarly secured to the end walls of plating tank 10, but at a slightly lower height, by braces 30. Anode hangers 20 and cathode hangers 24 are insulated with an inert coating, such as a vinyl plastisol insulation, over their entire surface except at the points of contact with the support rods and with the anode or cathode.

It is a critical feature of this invention that roll 16 be mounted so that it is only partially submerged in electrolyte solution 12, i.e., so that part of roll 16 is below the free surface of electrolyte solution 12 (the term "free surface" being used herein and in the appended claims to mean the upper surface of the solution when it is in a quiescent state) and the remaining part is above the free surface of electrolyte solution 12 and thus exposed to the surrounding atmosphere. Considerable variation in the exact position at which roll 16 is mounted is, however, permissible. Specifically, roll 16 should be mounted with its axis substantially parallel to the free surface of electrolyte solution 12 and preferably at such a level that about 40 to about 90 percent of the total surface area of roll 16 is immersed within electrolyte solution 12 when it is in a quiescent state. It is particularly preferred that roll 16 be mounted so that from about 50 to about 75 percent of the total surface area thereof is immersed within electrolyte solution 12.

As shown in FIG. 2, the electric current required for the process is provided by a conventional direct current source, indicated by the numeral 32, such as a low voltage high amperage generator or rectifier, connected by power supply lines 34 and 36 to anode hangers 20 and cathode hangers 24 which serve to convey the current.

As shown in FIG. 3, electrolyte solution 12 is withdrawn from tank 10 via outlet pipe 38 and pumped by means of pump 40 through filter 42 and heat exchanger 44 and then back into tank 10 via inlet pipe 46. By this means, continuous recirculation of electrolyte solution 12 throughout the plating process is achieved and substantially uniform conditions are maintained throughout plating tank 10.

As shown in FIG. 4, agitation of electrolyte solution 12 is effected by means of sparging pipe 48 which is of a length comparable to roll 16 and is provided with a series of orifices 50, which may take the form of slots or holes, spaced at equal increments along its longitudinal axis. Sparging pipe 48 is closed at one end by cap 52 and connected at its other end to high capacity blower 54 which serves to provide the air required for sparging. Blower 54 can, of course, be replaced by any other suitable source of air which will maintain an adequate volumetric flow rate to effectively agitate electrolyte

solution 12 and which provides air which is free of oil or other contaminants. As illustrated, sparging pipe 48 is positioned in the bath so that it is immediately below and substantially parallel to roll 16 so that the streams of bubbles 51 emerging from orifices 50 and rising through electrolyte solution 12 will uniformly contact the surface of roll 16. To provide for rotation of roll 16 about its axis during the plating process, variable speed motor 56 is connected by way of drive shaft 58, which extends through a seal in the wall of tank 10, and coupling 60 to shaft section 18 at one end of roll 16. An alternative method which avoids the problems encountered in providing a seal in the wall of a tank containing a corrosive liquid is to employ a submerged motor drive positioned within tank 10. Various other means of providing for rotation of roll 16 would be apparent to one skilled in the art.

In operating the apparatus of this invention, roll 16, which is to be plated with nickel, is mounted in position within tank 10 and connected to the drive shaft of motor 56 which is then started so as to rotate roll 16 about its axis. Blower 54 is then put into operation with the result that a continuous stream of bubbles 51 rises from each of slots 50 in sparging pipe 48 and breaks over roll 16 causing electrolyte solution 12 to be violently agitated and carried up and over the exposed surface of rotating roll 16 so as to keep such surface completely and continuously covered with a layer of electrolyte solution 12. At the same time, pump 40 is started so as to circulate electrolyte solution 12 through filter 42 and heat exchanger 44, whereby electrolyte solution 12 is maintained substantially free from solid contaminants and at the temperature required for the plating operation. As the flow of electric current from power supply source 32 is started, formation of a nickel plate on the surface of roll 16 begins and operation is continued until the desired thickness of nickel plate is achieved, whereupon the apparatus is shut down and roll 16 is removed from tank 10. Before plating a second roll, additional nickel chunks will, if necessary, be added to the perforated cylinders of anodes 14.

The method of this invention is applicable to plating of many different types of cylindrical objects regardless of their size, or whether they are solid or hollow, or composed of any particular material, so long as such material is capable of being metal plated in an electroplating process. While the invention is described herein with particular reference to the plating of a cylinder, and will ordinarily find its most widespread application in the plating of cylinders, it can also be employed in plating other elongated bodies which are not of circular cross-section. Thus, for example, the object to be plated may have a cross-sectional configuration which takes the form of an oval, an ellipse, or a polygon. All such objects are intended to be included within the scope of the term "an object of generally cylindrical shape" as employed herein and in the appended claims. Moreover, if a cylinder is provided with shaft sections at its ends, as is frequently the case, then these sections will also be plated as will the entire ends of the cylinder. If plating of these areas is not desired then they may, of course, be provided with protective coverings to prevent plating, but it is ordinarily desirable to plate both the shaft sections and the ends of the cylinder and in such instances the method of this invention provides an important advantage over prior art methods, such as the method disclosed in U.S. Pat. 1,918,627, in which this is not accomplished. Although it has been specifically illustrated herein with reference to nickel plating, the method of this invention is applicable to plating with other metals so long as the plating system is not one in which vigorous agitation of the electrolyte is detrimental, as is the case, for example, in chromium plating. Thus, for example, the method and apparatus described herein may be employed to carry

out silver plating, zinc plating, or copper plating of cylindrical objects, as well as nickel plating.

As pointed out hereinbefore, the cylindrical object which is to be plated is mounted so that its axis is substantially parallel to the free surface of the electrolyte solution and either coincident with or spaced therefrom so that a portion of the object is immersed in the solution and the remaining portion extends above the free surface of the solution. The optimum position for the cylindrical object will depend on a number of factors, particularly the diameter of the object and the degree of agitation imparted to the electrolyte solution. As indicated hereinbefore, it is preferred in practicing this invention that about 40 to about 90 percent of the total surface area of the object be immersed when the electrolyte solution is in a quiescent state and particularly preferred that about 50 to about 75 percent be immersed. With cylindrical objects of small diameter, such as 2-inch diameter rolls, a position where the axis is coincident with the free surface, i.e. 50 percent of the total surface area immersed, is ordinarily optimum, whereas larger cylindrical objects, such as 8-inch diameter rolls, will usually require a greater degree of immersion. Generally speaking, the greater the diameter of the object the more it should be immersed so as to ensure that the agitation of the bath will be effective to maintain an adequate flow of electrolyte solution over the exposed portion of the object.

To maintain the electrolyte solution at a substantially uniform concentration and temperature at all points within the bath it is desirable to continuously recirculate a portion of the solution. Such recirculation can be accomplished by the use of any suitable pumping means known to the art. In nickel electroplating with the process of this invention, the recirculation rate should be sufficient to circulate each hour a volume of electrolyte solution which is equal to at least the total volume of solution in the tank, i.e. a tank "turnover" rate of at least one time per hour, and preferably equal to at least 1.5 times the total volume of solution in the tank. Moreover, since some loss of electrolyte solution will inevitably occur due to evaporation and/or leakage, "make-up" solution should be added during the plating process. It is also desirable to maintain the electrolyte solution at a constant level in the plating tank and for this purpose a weir (not shown in the drawing) is preferably provided at one end of the tank. The circulating system can then be arranged to remove some solution from near the bottom of the plating tank and some from the weir box. Any other suitable arrangement for maintaining a constant level of solution in the plating tank can, of course, be employed in place of a weir.

The temperature of the electroplating bath is not ordinarily critical but it will frequently be desirable to provide means for heating the electrolyte solution so that operation at temperatures above room temperature is rendered possible. In nickel electroplating with the process of this invention, it is desirable to maintain the bath at a temperature in the range of about 100° F. to about 175° F., and preferably in a range of about 120° F. to about 150° F. Any conventional means of providing the necessary heat input may be employed, for example, the plating tank may be jacketed and a suitable heat transfer fluid passed through the jacket, or, in recirculating, the electrolyte solution may be passed through a heat exchanger where the temperature is raised to the necessary level before it is returned to the plating tank. In addition to heating the electrolyte solution to maintain a desirable temperature for plating, it is also advantageous that the circulation system include a filter to effect removal of any solid particles which are present in the electrolyte solution. Any conventional type of filter may be employed, but in nickel electroplating with the method of this invention it is preferred to employ a filter capable of retaining one hundred percent of the particles greater than five microns in size.

As will be apparent from the foregoing disclosure, the essential requirements of the method of this invention are (1) that the cylindrical object be properly positioned with reference to the level of electrolyte solution, as hereinbefore described, and (2) that the electrolyte solution be agitated with sufficient force that it washes over the portion of the cylindrical object extending above the free surface of the electrolyte solution, so as to scrub this portion, yet maintains this portion continuously and completely covered to an extent adequate to ensure that plating occurs thereon. It will ordinarily also be highly advantageous to rotate the cylindrical object about its axis so as to ensure uniformity of plating and the preferred embodiments of this invention include such rotation. However, the method of this invention is operable without such rotation, particularly where completely uniform plate thickness is not essential, since by maintaining the exposed surface of the object completely awash with electrolyte solution plating is taking place over the entire surface throughout the entire plating period and it is thus not necessary to rotate in order to effect plating of the entire surface. In contrast with the method of the prior art in which the cylinder is partially immersed so that plating action takes place only in the region of immersion and the purpose of rotating the cylinder is to effect plating of the entire surface, in the method of this invention plating action is taking place at all times over the entire surface of the cylinder and the purpose of rotating is to compensate for the fact that all points on the plating surface are not equidistant from the anode so as to provide a plate of uniform thickness in spite of the lack of equidistant spacing.

Consonant with the above requirements, many variations and modifications in the method of this invention are feasible. Thus, for example, rotation of the cylindrical object may be continuous, or it may be intermittent with a short interval during which the cylinder is stationary between each period of rotation, or it may be incremental in nature with the cylinder being turned successively by a quarter turn or a half turn each time. The exact speed of rotation is not critical, but it is preferred in electroplating with nickel to employ a speed of 5 to 10 revolutions per minute.

The required agitation of the electrolyte solution can be accomplished by any suitable means as long as the solution is agitated with sufficient force to continuously and completely cover the portion of the cylindrical object above the quiescent level of the bath with a layer of electrolyte solution of adequate thickness, for example, one quarter inch or more, to ensure that electrolytic deposition can occur at all points on the surface defined by the rotating cylinder. In other words, the agitation must be such that the solution rolls over the rotating cylinder and keeps its upper surface awash at all times. This provides the desired scrubbing action at the surface of the cylinder while at the same time ensuring that plating current is carried to all portions of the cylinder at all times. Such agitation may be accomplished by sparging with air or other inert gas such as argon or nitrogen, by solution sparging, i.e. by injecting streams of electrolyte solution through a multiplicity of jets located within the bath directly below the rotating cylinder, or by mechanical stirring such as by the use of paddle wheels located near the rotating cylinder.

It is preferred to effect agitation of the electrolyte solution by means of gas sparging and particularly preferred to employ large bubble air sparging. Such preference is dictated in part by the fact that sparging is a simple, convenient and low cost method but also by the fact that it provides for a desirable heterogeneity in the conditions at the surface of the cylinder, i.e. since the rising bubbles travel along constantly fluctuating paths there is continual variation in the scrubbing action at the surface of the cylinder which is particularly effective in dislodging particles and provides excellent uniformity of plating and freedom from "in plate" defects. The most effective scrub-

bing action is achieved by providing for the formation of large bubbles which rupture violently at the surface. Large bubble air sparging is most conveniently and inexpensively accomplished by inserting a sparging pipe into the bath immediately below the rotating cylinder and providing such pipe with a series of longitudinally spaced slots or holes so that a substantially uniform stream of air bubbles will rise along the length of the sparging pipe and cause the electrolyte solution to constantly roll over the rotating cylinder. The sparging pipe is preferably located so that it is parallel to and in line with the longitudinal axis of the cylinder and at a distance of about 2 to about 8 inches below the bottom surface of the cylinder. The slots or holes should be of such size that the air bubbles will be at least  $\frac{1}{2}$ -inch in diameter, and preferably larger, when they break at the surface, as this provides the most effective scrubbing action. Satisfactory results are obtained by the use of, for example,  $\frac{1}{32}$ -inch diameter holes spaced 1.3 inches apart. The air supplied to the sparging pipe should be pressurized, with the optimum pressure depending on the position of the pipe within the bath. Good results are obtained by providing a pressure of about one p.s.i.g. for each 18 inches of solution above the top surface of the sparging pipe. The volume of air required for sparging will, of course, depend upon the specific geometry of the plating system involved, but, in general, should be at least 2 cubic feet per minute for each square foot of surface being plated, and preferably 3 to 4 cubic feet per minute for each square foot of surface.

30 The plating tank may be of any convenient geometry but will ordinarily be of a rectangular shape. The anodes may also be of any suitable shape but must be positioned in the tank in such manner that they do not interfere with the sparging pipe, or other agitating means, and should be arranged so as to provide a "live" anode surface extending longitudinally over at least the central three-quarters of the cylinder.

A convenient and effective procedure is to utilize anodes in which the plating metal is in the form of chunks carried 40 in perforated baskets which are suspended in the electrolyte solution, as illustrated herein. However, other conventional types of anode construction may also be employed, for example, the anode may be a horizontally positioned perforated basket of comparable length to the cathode which is immersed in the electrolyte solution and supported in proximity to the cathode. Any conventional anode construction would be permissible in carrying out the method of this invention so long as the anode is disposed so as to be effective over the full length of the object being plated and does not interfere with the gas sparging or other means employed for agitating the electrolyte solution. Moreover, the anode need not be a soluble anode as illustrated herein but may be an inert or insoluble anode, in which instance the plating metal would be supplied from the electrolyte. Thus, for example, nickel plating can be effected using a suitable solution of soluble nickel salts as the electrolyte and an insoluble anode composed of lead, platinum, platinized titanium, or graphite.

60 The optimum current density for operation of the process will depend upon the specific situation involved, including such factors as the composition and temperature of the bath, the relative positions of anode and cathode, and so forth. It has been found that current densities of 50 to 100 amperes per square foot of plating surface, or more, are ordinarily feasible in nickel plating in the manner described herein.

65 The method of this invention is particularly amenable to the production of a hard nickel plate such as is required for film transport rolls used in the manufacture of photographic film. To produce a bright, hard and tough nickel deposit, a typical plating bath will contain nickel sulfate hexahydrate and/or nickel sulfate heptahydrate in an amount of about 24 to about 48 ounces per gallon, nickel chloride in an amount of about 4 to about 6 ounces per

gallon, boric acid in an amount of about 4 to about 5 ounces per gallon, saccharin in an amount of about 0.2 to about 0.4 ounce per gallon, ammonium bifluoride in an amount of about 0.2 to about 0.4 ounce per gallon, and a low foaming surfactant in an amount sufficient to provide a surface tension of less than about 45 dynes per square centimeter. Where it is desired to produce a soft nickel deposit, this may be readily accomplished by using a similar plating bath in which the saccharin is omitted.

The method of this invention provides a very high plating rate while at the same time providing a very high quality plate. Thus, in nickel electroplating using a free dissolving form of electrolytic nickel plating rates of from about 0.004 inch per hour to as high as about 0.006 inch per hour can be attained. These rates are achieved primarily as a result of the fact that the vigorous agitation provided results in adequate replenishment of the electrolyte surface film at the cathode to sustain a high plating rate. Furthermore, the nickel plate is substantially improved over that obtained by methods heretofore known with respect to the presence of "in plate" defects. Such defects are substantially eliminated, or at least greatly reduced in number, as a result of the washing action of the electrolyte solution over the surface of the cylinder. Also, since the cylinder is positioned so that it is only partially immersed, "gravity head" of electrolyte solution over the cylindrical surface is substantially eliminated so as to greatly minimize the settling out of solid particles onto the cylinder. Moreover, the violent agitation of the electrolyte solution causes it to constantly wash over the rotating cylinder and thereby scrub the surface so as to dislodge small bubbles and/or conductive solid particles which would otherwise be "plated in." The overall result of these features of the process is that a plate which is remarkably free of defects, and thus well suited to applications requiring stringent quality standards such as plating of film transport rolls, is produced.

Apparatus constructed in accordance with the disclosure herein was operated to nickel plate film transport rolls with excellent results. Both 4-inch diameter by 48-inch long steel rolls and 2-inch diameter by 48-inch long aluminum rolls were plated at a current density of 75 amperes per square foot. The plating bath was maintained at a pH of approximately 4 and a temperature of approximately 145° F. and contained 24 ounces per gallon of a mixture of nickel sulfate hexahydrate and nickel sulfate heptahydrate, 6 ounces per gallon of nickel chloride, 5 ounces per gallon of boric acid, 0.3 ounce per gallon of saccharin, 0.2 ounce per gallon of ammonium bifluoride, and sufficient low foaming surfactant to maintain the surface tension below 45 dynes per square centimeter. The bath was recirculated at a rate sufficient to turn the solution over about 1.5 times per hour and passed through a filter which retained all particles above 5 microns in size. The roll was suspended in the bath so that it was a little more than half immersed in the electrolyte solution and was adjacent to an anode consisting of 1" x 1" x 1/2" nickel chips contained in 2 1/2-inch diameter by 24-inch long perforated titanium baskets. Rotation of the roll was at a rate of 7 1/2 revolutions per minute with large bubble air sparging at a rate sufficient that the electrolyte solution was violently agitated and washed over the rotating roll at all times. A plating rate of about 0.006 inch per hour was achieved and the resulting plate was uniform in thickness, bright, hard, and abrasion resistant and almost completely free of "in plate" defects.

The invention has been described in detail with particular reference to preferred embodiments thereof, but it will be understood that variations and modifications can be effected within the spirit and scope of the invention as described hereinabove and as defined in the appended claims.

We claim:

1. In a method of metal electroplating wherein the object to be plated is either a cylinder or of a generally 75

cylindrical shape, said object serves as cathode in the plating process and is positioned adjacent to an anode which is immersed within an electrolyte solution, and an electric potential is impressed across said anode and said object to effect plating; the improvement comprising partially immersing the object in the electrolyte solution with its longitudinal axis substantially parallel to the free surface of the electrolyte solution so that a portion of the object is below said free surface and within the electrolyte solution and the remaining portion of the object extends above said free surface, and agitating the electrolyte solution during plating of the object by sparging with a fluid introduced into the electrolyte solution directly beneath the object with sufficient force that the electrolyte solution washes over the portion of the object extending above said free surface to maintain said portion continuously and completely covered with electrolyte solution to an extent adequate to ensure that plating occurs thereon.

2. The method as described in claim 1 further comprising the step of rotating said object about said longitudinal axis during plating.

3. The method as described in claim 2 wherein the rotation is continuous.

4. The method as described in claim 2 wherein the rotation is intermittent.

5. The method as described in claim 2 wherein said object is positioned so that from about 40 to about 90 percent of the total surface area thereof is immersed within said electrolyte solution when said electrolyte solution is in a quiescent state.

6. The method as described in claim 2 wherein said object is positioned so that from about 50 to about 75 percent of the total surface area thereof is immersed within said electrolyte solution when said electrolyte solution is in a quiescent state.

7. The method as described in claim 2 wherein said object is plated with nickel.

8. The method as described in claim 2 wherein said object is plated with copper.

9. The method as described in claim 2 wherein said object is plated with zinc.

10. The method as described in claim 2 wherein said object is plated with silver.

11. The method as described in claim 2 wherein the agitation of said electrolyte solution is accomplished by sparging with an inert gas.

12. The method as described in claim 11 wherein the gas is introduced into the electrolyte solution from a sparging pipe having a series of longitudinally spaced orifices in the wall thereof which is positioned directly below and parallel to said object and at a distance of about 2 to about 8 inches therefrom.

13. The method as described in claim 12 wherein the gas is introduced into the electrolyte solution at a rate of at least about 2 cubic feet per minute for each square foot of surface plated.

14. Apparatus for electroplating with a metal coating an object which is either a cylinder or of a generally cylindrical shape, comprising:

(1) a tank containing a body of electrolyte solution having a free upper surface,

(2) an anode immersed within said electrolyte solution,

(3) means for mounting the object adjacent said anode with the longitudinal axis of the object substantially parallel to the free surface of said electrolyte solution in such position that a portion of the object is below said free surface and within the electrolyte solution and the remaining portion of the object extends above said free surface,

(4) a sparger positioned within said electrolyte solution for introducing a sparging fluid during plating of the object into said electrolyte solution directly beneath the object with sufficient force that said electrolyte solution washes over the portion of the object extending above said free surface to maintain

## 11

said portion continuously and completely covered with electrolyte solution to an extent adequate to ensure that plating occurs thereon, and  
(5) means for impressing an electric potential across said anode and said object.

15. Apparatus as described in claim 14 wherein said object is rotatably mounted and including means for rotating said object about its longitudinal axis.

16. Apparatus as described in claim 15 wherein said sparger is a gas sparging pipe.

17. Apparatus as described in claim 16 wherein said pipe has a series of horizontally spaced orifices in the wall thereof and is positioned within said electrolyte solution directly below and parallel to said object and at a distance of about 2 to about 8 inches therefrom.

18. Apparatus as described in claim 17 wherein said orifices are of such size that bubbles which are at least about one-half inch in diameter when they reach the surface of said electrolyte solution are formed.

19. Apparatus as described in claim 15 including means for recirculating a portion of said electrolyte solution.

20. Apparatus as described in claim 15 including means for heating said electrolyte solution.

21. Apparatus as described in claim 15 including means for filtering said electrolyte solution to remove solid particles therefrom.

22. Apparatus as described in claim 15 wherein said anode is an insoluble anode.

23. Apparatus as described in claim 15 wherein said anode is a soluble anode.

24. Apparatus as described in claim 23 wherein said anode is a nickel anode.

25. Apparatus as described in claim 23 wherein said anode is a copper anode.

26. Apparatus for electroplating a cylinder with a nickel coating, comprising:

(1) a tank containing a body of electrolyte solution having a free upper surface,

(2) an anode of free dissolving electrolytic nickel mounted so that it is immersed within said electrolyte solution,

(3) means for rotatably mounting said cylinder adjacent said anode with its longitudinal axis substantially parallel to the free surface of said electrolyte

## 12

solution in such position that about 50 to about 75 percent of the total surface area of said cylinder is immersed in said electrolyte solution when said electrolyte solution is in a quiescent state and the remaining portion of said cylinder extends above said free surface,

(4) means for rotating said cylinder about its longitudinal axis,

(5) a sparging pipe positioned within said electrolyte solution directly below said cylinder for agitating said electrolyte solution during plating of said cylinder so that it washes over the portion of said cylinder extending above said free surface to maintain said portion continuously and completely covered with electrolyte solution to an extent adequate to ensure that plating occurs thereon,

(6) a source of air connected to said sparging pipe,

(7) a pump for recirculating a portion of said electrolyte solution,

(8) a filter through which said electrolyte solution is passed to remove solid particles therefrom,

(9) means for heating said electrolyte solution, and

(10) means for impressing an electric potential across said anode and said cylinder.

## References Cited

## UNITED STATES PATENTS

|           |         |          |         |
|-----------|---------|----------|---------|
| 1,249,787 | 12/1917 | Leuchter | 204—277 |
| 1,423,815 | 7/1922  | Park     | 204—277 |
| 1,473,060 | 11/1923 | Taylor   | 204—277 |
| 1,884,512 | 10/1932 | Ballard  | 204—25  |
| 2,155,392 | 4/1939  | Ballard  | 204—25  |
| 2,435,872 | 2/1948  | Coulson  | 204—25  |

## FOREIGN PATENTS

|         |        |         |         |
|---------|--------|---------|---------|
| 873,926 | 3/1954 | Germany | 204—25  |
| 631,672 | 4/1963 | Belgium | 204—212 |

JOHN H. MACK, Primary Examiner

T. TUFARIELLO, Assistant Examiner

## U.S. CL. X.R.

204—212, 273, 275, 277